

## UNITED STATES PATENT OFFICE.

SHINJIRO HORII, OF TOKYO, JAPAN.

## STENCIL SHEET.

No Drawing. Application filed December 3, 1925. Serial No. 73,060.

This invention relates to improvements in stencil sheets of the type commonly used for autographic and typewriting duplication, consisting of a sheet of fibrous material 5  
coated or impregnated with a composition comprising esters of polysaccharides, naphthenic acids for the purpose of preparing the superior stencil sheets which offer a considerably great resistance to the atmospheric influences on using or storing, and give a 10  
larger number of clear and sharp copies.

It is well known that a solution of colloidion or celluloid, combined with castor oil or other fatty oils as a tempering agent, 15  
has been used for a coating material to produce stencil sheets. Such a composition does not, however, produce a superior stencil sheet, having the disadvantages of being sticky on handling and, moreover, the 20  
coated medium is not soft enough to give a clear writing by the abrasion of a stylus or by the impact of the type of a writing machine.

It has been found that it is possible to 25  
incorporate uniformly the cellulose esters into naphthenic acids, and that the composition comprising esters of polysaccharides, combined with naphthenic acids is the most superior coating material for stencil sheets, 30  
which gives a coating of the desired uniform softness but without the stickiness and is not brittle in cold weather. The stencil sheets thus obtained can be used throughout 35  
an extended period of time without any change on the coating and produce therefrom a large number of clear and sharp copies.

In carrying out the invention a sheet of 40  
fibrous material, for instance Yoshino paper, is coated or impregnated with a coating solution prepared by dissolving esters of polysaccharides, such as starch acetates, cellulose acetates, cellulose nitrates and cellulose xanthate, in suitable solvents, such as alcohols, acetone, theylacetate, amylacetate ether, 45  
and adding naphthenic acids. To the above

mentioned composition, if desired, may be added fatty acids, fatty oils, fats and waxes, such as castor oil, Japan wax, ceresin, as tempering agents. Or this composition may 50  
be added into the paper stuff in a mixing hollander.

The proportions of the ingredients of the composition may vary according to several circumstances, but an example is as follows:—

| Parts by weight.           |    |    |
|----------------------------|----|----|
| Nitrocellulose (pyroxylin) | 5  |    |
| Naphthenic acids           | 10 |    |
| Japan wax                  | 5  | 60 |
| Methanol                   | 15 |    |
| Aceton                     | 15 |    |
| Amylalcohol                | 30 |    |

As stated the coated sheets remain 65  
throughout an extended period of time practically unchanged without the drawback of becoming sticky or friable on handling or storing. By the abrasion of a stylus or the blow of the type of a typewriter, without 70  
necessity of moistening the sheets with water or moistening solutions, the clear characters may be easily produced thereon.

The term "esters of polysaccharides" is intended to include not only one of definite 75  
esters of polysaccharides, but also a mixture of them.

What I claim is:—

1. A stencil sheet adapted for stencilizing by pressure, comprising a base of fibrous 80  
material impregnated with a composition including esters of polysaccharides, and naphthenic acids.

2. A stencil sheet adapted for stencilizing by pressure, comprising a base of fibrous 85  
material impregnated with a composition including esters of polysaccharides, naphthenic acids and tempering agents, such as fatty acids, fatty oils, fats and waxes.

In testimony whereof I affix my signature.

SHINJIRO HORII,